# EUROPEAN PATENT SPECIFICATION

(11) **EP 0 270 265 B1**
(45) Date of publication and mention of the grant of the patent: **01.07.1992**
(21) Application number: 87309972.5
(22) Date of filing: 11.11.1987
(51) Int. Cl.: C23C 4/12, C22C 1/10

(54) **Making composite metal deposit by spray casting**
Verfahren zur Herstellung von Verbundwerkstoffen durch Aufsprühen von geschmolzenem Metall
Fabrication d'un composite métallique par pulvérisation de métal liquide

(30) Priority: 14.11.1986 GB 8627308
(43) Date of publication of application: 08.06.1988
(73) Proprietor: ALCAN INTERNATIONAL LIMITED, Montreal Quebec H3A 3G2 (CA)
(72) Inventor: Jordan, Richard Michael, Hook Norton Oxon OX15 5NX (GB)
(74) Representative: Wilkinson, Stephen John

(56) References cited:
- DE-A- 2 439 620
- FR-A- 2 156 889
- FR-A- 2 311 101
- GB-A- 1 083 003
- GB-A- 1 410 169
- GB-A- 1 531 222
- US-A- 2 993 264
- US-A- 3 826 301
- PATENT ABSTRACTS OF JAPAN, vol. 7, no. 268 (C-197)[1413], 30th November 1983; & JP-A-58 147 556 (HITACHI SEISAKUSHO K.K.) 02.09.1983

## Description

This invention is concerned with a method of making a composite metal deposit by spray casting. The technique of spray casting is well known and comprises the steps of atomising a stream of molten metal to form a spray of hot metal particles by subjecting the stream to a relatively cold gas directed at the stream, and depositing the spray on a substrate. The provision of rapid and controlled cooling permits the production of deposits having unusual microstructures, which can be rolled or formed into shaped articles. But with only one source of molten metal, there is a limit to the range of compositions and microstructures that can be obtained.

US Patent No 4674554 describes a spray casting method which includes the step of applying to the stream or spray fine, solid particles of a material of different composition from the metal. The particles are incorporated in the deposit. The use of refractory particles e.g. of alumina or silicon carbide can result in metal matrix composites having enhanced properties.

US Patent 4522784 describes a casting method in which two streams of molten metal are mixed just prior to casting, the smaller stream having a higher temperature than the larger stream and being chosen so that a fine intermetallic precipitate is formed during and prior to casting. With the DC casting methods described, it is difficult to remove heat fast enough from the system to prevent to resolution of the intermetallic precipitates.

GB 1359486 describes a spray casting technique for casting two immiscible metals of different density. A single flow of molten metal consisting of concentric streams of the two metals is atomised and the drops collected on a substrate. The range of alloy compositions that can be cast in this way is quite restricted.

This invention provides a convenient way of making composite metal deposits by spray casting, which is characterized over the above prior art by the fact that separate streams of molten metal are atomised separately. As a result, there is much less restriction on the compositions of the two metals.

GB 1083003 describes a method of making bearing materials by spraying Al and Pb simultaneously onto a backing strip. This results in a microstructure comprising alternating regions, of size corresponding (substantially) to the molten spray droplets, of Al and Pb. US 3826301 contains a similar disclosure.

The invention provides a method of making a laminated metal article having consecutive layers of deposited metal compositions wherein the compositions of any two consecutive layers in the laminated article are different which method comprises providing at least two metal streams and a substrate, atomising each of the metal streams to form at least two sprays of hot metal particles by subjecting each of the metal streams to relatively cold gas directed at the said metal streams, depositing metal particles from one of the said streams onto the substrate to form a first layer thereon, depositing metal particles from another of the same metal streams onto the first layer to form a second layer and, if desired, depositing in a consecutive manner layers of metal particles from any of the said sprays such that any two consecutive layers have different compositions whereby a laminate is produced, wherein the atomisation conditions are controlled such that the metal particles of the sprays are partially or fully liquid but supercooled on impact to the extent that solidification takes place immediately on impact or that deposition on the substrate is followed by immediate solidification.

The first and second metal streams may be provided by gravity flow from holding vessels containing supplies of the molten metals. The invention contemplates the use of two, three or more molten metal streams, each being atomised separately, and references to first and second metal streams should be construed accordingly.

Atomisation conditions may be chosen, as is known in the art, to control the size, velocity, direction and temperature of the sprays of hot metal particles. On being atomised, the particles of molten metal spread out in a conical spray pattern, which may be of circular cross-section or may be modified, as known in the art, to form a different cross-section or a more even spread of metal particles.

The substrate may be a metal surface, which may for example be flat or tubular with the metal spray to be deposited on the inner or the outer surface. It is generally preferred that the metal particles be still at least partially liquid on impact, otherwise the deposit may be too porous. By suitable control of the atomising conditions, the metal spray is partially or fully liquid but supercooled on impact, so that solidification takes place immediately on impact and there is no need to extract large amounts of heat through the substrate.

It is possible to provide fibres, whiskers or particles of refractory material, e.g. carbon or silicon carbide, on the substrate in such a way that they become embedded in the coherent composite metal deposit and provide reinforcement for it. Also if desired, particles of refractory material can be incorporated in the first and/or second spray by the technique described in US-A-4674554 noted above.

Three (or more) sprays may be used. For example the spray patterns of two may be superimposed and operated simultaneously to form one layer of the laminate structure. The result, therefore, is a laminated structure in which alternate layers have a microstructure resulting from the two simultaneously operated sprays. Or two superimposed sprays may be chosen to interact as described in the aforesaid US patent 4522784.

There is no critical range of ratios of the two metals constituting the first and second sprays. Suitable proportions of the two (or more) metals are chosen for particular applications. The spray patterns of the first and second sprays may, but need not, overlap; that is to say, the two sprays may be arranged to impact on the same or different areas of the substrate. The substrate may be translated, or reciprocated, or rotated in order to pick up the two metal sprays. These features can be used to exercise further control over the structure of the deposit. For example, if the spray patterns of the two sprays do not overlap and the substrate is reciprocated between them, the deposit may consist of alternating layers of first and second metal.

If the spray patterns of the two sprays do overlap, then it is necessary to operate the two sprays alternatively in order to achieve the desired laminated structure. In order to operate both sprays continuously, it is therefore preferred that the two spray patterns can be arranged not to overlap, and to reciprocate or rotate the substrate so that alternating layers of the two metals are deposited thereon.

Other variations in structure can be achieved by supplying a first metal stream initially, followed by the second, so that the deposit consists of the first metal with a surface coating of the second. The supply of molten metal in two or more streams gives the operator a great deal of latitude in determining the structure of a deposit.

Preferably, the laminated deposit comprises at least two layers of each metal in alternating superimposed relationship. The thickness of the alternating layers has a significant effect on the properties of the laminate. In the as-sprayed deposit, each layer preferably has a thickness in the range 0.01-100 mm, particularly 1-10 mm. The as-sprayed deposit may be subjected to rolling. For many purposes it is preferred that each layer in the rolled product have a thickness of from 10 to 500 µm, particularly 30 to 200 µm.

Since the two metals do not contact one another prior to deposition on the substrate, which is followed by immediate solidification, there is very little restriction on the nature of the metals that may be used. It would be disadvantageous if the temperature of one metal on deposition were so high that substantial melting of the other took place on the deposit. It is often convenient to use two different alloys of the same base metal. The method is of particular interest for spray casting aluminium alloys, for which purpose an inert gas such as argon or nitrogen is generally desirable though not essential.

Reference is directed to Figures 1 to 3, each of which is a schematic diagram of a system for making a composite metal deposit according to the invention. Referring to Figure 1, the system comprises first and second furnaces 10 and 12 for supplying first and second streams of molten metal, which are atomised (by means not shown) to form first and second sprays, 14 and 16, of hot metal particles. The spray patterns overlap, and each spray is operated in turn while the other is shut off. The sprays are deposited in turn on a substrate 18, whose position and orientation are controlled by means 20. The metal sprays and the substrate are contained within a spray chamber 22, which is closed except for an exit vent for gas and any overspray powder.

A refractory material contained in a stream of carrier gas is supplied via a pipe 26 to the region where the first metal is atomised, and becomes incorporated in the first metal spray 14.

In the system shown in Figure 1, the substrate 18 might be maintained stationary, so as to build up a composite metal body thereon; or it might be translated, rotated or reciprocated in order to build up a uniform composite metal layer. The substrate 18 might have taken the shape of a mould, with the intention of working the deposit while on the substrate to form a shaped article.

Figure 2 corresponds to Figure 1, except that the spray patterns of the two metal sprays 14 and 16 are shown as being non-overlapping. In this case, the sprays are operated continuously and the substrate 18 is reciprocated in order to obtain a deposit consisting of alternating layers of first and second metal.

In Figure 3, the spray patterns of the two metal sprays 14 and 16 are shown as partly overlapping when they impact on cylindrical substrate 18 which is caused to rotate round a horizontal axis 28. A fibre 30 is supplied from a spool 32 and becomes incorporated in the deposit.

There follows examples of combinations of metals and alloys that can be used to make composite metal deposits according to this invention. In each case, the first metal or alloy mentioned will generally be present in the deposit in a volume concentration as great or greater than the second metal or alloy.
A. The first metal is the alloy designated 7010 in the Aluminium Association Register, and the second metal is a softer Al alloy such as 6061 or pure Al metal. 7010 is typically used for aircraft structures, and the second metal improves fracture toughness by a micro-laminated structure to reduce fatigue and blunt cracks.
B. The first metal is 7010 alloy and the second metal is 6010 alloy to confer ductility, toughness and fatigue resistance.
C. The first metal is 7010 alloy and the second metal is an Al/Zn alloy to improve stress corrosion resistance.
D. The first metal is 7075 alloy, used for armour plating, and the second metal is an Al/Si alloy to increase resistance to spalling.
E. The first metal is 7075 alloy, and the second metal is Pb to increase density, improve ballistic properties, and provide a microstructure to break up shock waves.
F. The first metal is any Al alloy and the second metal is Zn, applied on the surface as a layer amounting to 1 to 5% of the total thickness of the deposit, to aid diffusion bonding.
G. The first metal is 6061 alloy and the second metal is 7475 alloy + SiC to provide a product having improved ductility and toughness.

### EXAMPLE

Laminated material was sprayed using a combination of 6061 Al alloy from on atomizer and 7475 Al alloy + SiC from the other atomizer.

### 1. Spraying conditions.

Both crucibles used were alumina with zirconia nozzles. The atomizing gas was nitrogen. The collector was an aluminium plate 300 mm long by 150 mm wide. The plate was reciprocated beneath the sprays at a frequency of 1Hz.

The conditions for the 7475 alloy were the same apart from the melt temperature which was 710°C. SiC particulate (F600) was fed to the 7475 spray only, SiC was fed at a rate of 1.72 kg/min to the atomizing nozzle.

Several batches of material were made using similar conditions.

### 2. Microstructure of product

Measurements of the elemental distribution across the bands indicate that there has been a degree of interdiffusion between adjacent layers indicating that an effective metallurgical bond has been made between them. The SiC content of the 7475 layers was 10-12% by volume.

### 3. Mechanical properties

The as - sprayed material was consolidated by hot rolling at 430°C to approximately 2 mm in thickness and then further cold rolling to 1 mm. Any as - sprayed porosity was found to close up during this process to form a fully consolidated product. The sheet was solution heat treated by holding for at least 30 min at 500°C and cold water quenching. The material was artificially aged for 20 hr at 120°C.

Tensile properities were determined on several batches of sheet containing different thicknesses of laminate. The following table contains a summary of the results.

Crack initiation and propagation were also determined with the following results.

These results illustrate that the combination of the two materials in the laminate can result in improvements in mechanical properties over the individual constituents. In this instance the results indicate an improvement in strength and ductility over 6061 and an improvement in ductility and crack initiation and propagation energy (indicating improved toughness) over the 7475 alloy with SiC. The results also indicate a significant improvement in the properties (notably ductility) over that of the 6061 alloy with SiC. It is also notable that the thickness of the laminated regions is highly important in controlling the final properties of the material - specifically in this instance the ductility and toughness of the laminate.

## Claims

1. A method of making a laminated metal article having consecutive layers of deposited metal compositions wherein the compositions of any two consecutive layers in the laminated article are different which method comprises providing at least two metal streams and a substrate, atomising each of the metal streams to form at least two sprays of hot metal particles by subjecting each of the metal streams to relatively cold gas directed at the said metal streams, depositing metal particles from one of the said streams onto the substrate to form a first layer thereon, depositing metal particles from another of the said metal streams onto the first layer to form a second layer and, if desired, depositing in a consecutive manner layers of metal particles from any of the said sprays such that any two consecutive layers have different compositions whereby a laminate is produced, wherein the atomisation conditions are controlled such that the metal particles of the sprays are partially or fully liquid but supercooled on impact to the extent that solidification takes place immediately on impact or that deposition on the substrate is followed by immediate solidification.

2. A method as claimed in claim 1, wherein there are provided fibres, whiskers or particles of refractory material on the substrate in such a way that they become embedded in the coherent composite metal deposit.

3. A method as claimed in claim 1, wherein particles of a refractory material are applied to at least one of the metal streams or to at least one of the sprays of hot metal particles.

4. A method as claimed in claim 1, wherein two metal streams are used and particles of a refractory material are applied to one of the metal streams or to the spray formed from one of the metal streams such that a laminate is produced wherein consecutive layers of deposited metal do not both contain refractory particles.

5. A method as claimed in any one of claims 1 to 4, wherein the metals of the metal streams are different alloys of the same base metal.

6. A method as claimed in claim 5, wherein the base metal is aluminium.

7. A method as claimed in any one of claims 1 to 6, wherein there are provided two metal streams and wherein the laminated metal article comprises at least two layers of each metal in alternating superimposed relationship.

8. A method as claimed in any one of claims 1 to 7, wherein the laminated metal article is subsequently rolled.

9. A method as claimed in claim 8, wherein, after rolling, each deposited layer has a thickness of from 10 to 500 µm.

## Revendications

1. Procédé de fabrication d'un article métallique stratifié comportant des couches successives de compositions de métal déposées, les compositions de deux couches successives quelconques dans l'article stratifié, étant différentes, et ce procédé comprenant la mise en oeuvre d'au moins deux courants de métal et d'un substrat, l'atomisation de chacun des courants de métal pour former au moins deux jets de particules métalliques chaudes, en soumettant chacun des courants de métal à un gaz relativement froid dirigé vers ces courants de métal, en déposant les particules métalliques de l'un de ces courants, sur le substrat afin de former une première couche sur celui-ci, en déposant les particules métalliques de l'autre de ces mêmes courants de métal, sur la première couche pour former une deuxième couche et, si on le souhaite, en déposant successivement des couches de particules de métal à partir de l'un quelconque de ces jets de telle façon que deux couches quelconques successives, aient des compositions différentes, de sorte que l'on produit un stratifié ; les conditions d'atomisation étant ajustées de telle façon que les particules métalliques des jets, soient partiellement ou complètement liquides, mais sur-refroidies au moment de l'impact selon un degré tel que la solidification a lieu immédiatement au moment de l'impact, ou que le dépôt sur le substrat est suivi par une solidification immédiate.

2. Procédé selon la revendication 1, dans lequel on dépose des fibres, des trichites ou des particules de matériau réfractaire sur le substrat, de telle façon qu'elles soient incorporées dans le dépôt métallique composite cohérent.

3. Procédé selon la revendication 1, dans lequel des particules de matériau réfractaire sont introduites dans au moins un des courants de métal, ou dans au moins un des jets de particules métalliques chaudes.

4. Procédé selon la revendication 1, dans lequel on emploie deux courants de métal, et on introduit un matériau réfractaire dans l'un des courants de métal ou dans le jet formé à partir de l'un des courants de métal, de telle façon que l'on produise un stratifié dans lequel les couches successives de métal déposées, ne contiennent pas toutes les deux des particules réfractaires.

5. Procédé selon l'une quelconque des revendications 1 à 4, dans lequel les métaux des courants de métal, sont des alliages différents dérivés du même métal de base.

6. Procédé selon la revendication 5, dans lequel le métal de base est l'aluminium.

7. Procédé selon l'une quelconque des revendications 1 à 6, dans lequel on met en oeuvre deux courants de métal, et dans lequel l'article métallique stratifié comprend au moins deux couches de chaque métal alternativement superposées.

8. Procédé selon l'une quelconque des revendications 1 à 7, dans lequel l'article métallique stratifié est ensuite laminé.

9. Procédé selon la revendication 8, dans lequel, après laminage, chaque couche déposée, a une épaisseur de 10 à 500 µm.

## Patentansprüche

1. Verfahren zur Herstellung eines laminierten Metallartikels mit aufeinanderfolgenden Schichten von abgeschiedenen Metallzusammensetzungen, wobei die Zusammensetzungen von allen zwei aufeinanderfolgenden Schichten in dem laminierten Artikel verschieden sind, wobei das Verfahren umfaßt:
Das Zur-Verfügung-Stellen von wenigstens zwei Metallströmen und einem Substrat, Atomisieren jedes der Metallströme unter Ausbildung von wenigstens zwei Sprays von heißen Metallteilchen, indem man jeden der Metallströme einem relativ kalten Gas, welches auf die genannten Metallströme gerichtet ist, aussetzt, Abscheiden der Metallteilchen von einem der genannten Ströme auf das Substrat unter Ausbildung einer ersten Schicht darauf, Abscheiden der Metallteilchen von einem anderen der genannten Metallströme auf die erste Schicht unter Ausbildung einer zweiten Schicht und, gewünschtenfalls, Abscheiden in aufeinanderfolgender Weise von Schichten von Metallteilchen von allen der genannten Sprays derart, daß alle zwei aufeinanderfolgenden Schichten unterschiedliche Zusammensetzungen haben, unter Ausbildung eines Laminats, wobei die Atomisierungsbedingungen derart eingestellt werden, daß die Metallteilchen der Sprays teilweise oder vollständig flüssig, aber beim Auftreffen in einem solchen Maße unterkühlt sind, daß unmittelbar beim Auftreffen Verfestigung stattfindet, oder daß die unmittelbare Verfestigung im Anschluß an die Abscheidung auf dem Substrat erfolgt.

2. Verfahren gemäß Anspruch 1, bei dem Fasern, Whiskers oder Teilchen von feuerfestem Material auf dem Substrat derart vorgesehen sind, daß sie in der zusammenhängenden Verbundmetallabscheidung eingebettet werden.

3. Verfahren gemäß Anspruch 1, bei dem die Teilchen eines feuerfesten Materials in wenigstens einem der Metallströme oder in wenigstens einem der Sprays von heißen Metallteilchen eingebracht werden.

4. Verfahren gemäß Anspruch 1, bei dem zwei Metallströme verwendet werden, und Teilchen eines feuerfesten Materials in einem der Metallströme oder in den Spray, der sich aus einem der Metallströme bildet, derart eingebracht werden, daß ein Laminat ausgebildet ist, bei dem aufeinanderfolgende Schichten von abgeschiedenem Metall nicht beide feuerfeste Teilchen enthalten.

5. Verfahren gemäß einem der Ansprüche 1 bis 4, bei dem die Metalle der Metallströme unterschiedliche Legierungen des gleichen Grundmetalls sind.

6. Verfahren gemäß Anspruch 5, bei dem das Grundmetall Aluminium ist.

7. Verfahren gemäß einem der Ansprüche 1 bis 6, bei dem zwei Metallströme vorgesehen sind, und bei dem der laminierte Metallartikel wenigstens zwei Schichten des jeweiligen Metalls in alternierender, übereinanderliegender Beziehung umfaßt.

8. Verfahren gemäß einem der Ansprüche 1 bis 7, bei dem der laminierte Metallartikel anschließend gewalzt wird.

9. Verfahren gemäß Anspruch 8, bei dem nach dem Walzen jede abgeschiedene Schicht eine Dicke von 10 bis 500 µm hat.
